

Sept. 7, 1926.

1,598,683

G. W. HEISE

PROTECTED METALLIC ELECTRODE

Filed May 19, 1924

Fig. 1.



Fig. 2.



Inventor:

George W. Heise

By Bruce Townsend & Brickenstein

Attorneys.

## UNITED STATES PATENT OFFICE.

GEORGE W. HEISE, OF BAYSIDE, NEW YORK, ASSIGNOR TO NATIONAL CARBON COMPANY, INC., A CORPORATION OF NEW YORK.

## PROTECTED METALLIC ELECTRODE.

Application filed May 19, 1924. Serial No. 714,454.

This invention relates to improvements in protective coatings for those surfaces of metallic electrodes which are not required to be exposed to the electrolyte. The invention is particularly applicable in cells of the metal-caustic alkali-depolarizing oxid type. Reference will therefore be made primarily to this use, but it will be understood that the invention may be advantageously applied in other connections.

Caustic alkali cells ordinarily have a cathode comprising copper oxid or other depolarizing body, and an anode consisting of amalgamated zinc plates suspended in spaced relation on one or more sides of the cathode. Useful electrolytic action takes place chiefly between the cathode and the surfaces of the zinc opposed to it. The remaining zinc surfaces are subject to wasteful corrosion by local action, concentration effects, and other causes. The amount of zinc consumed in this manner may be a considerable proportion of the total amount used in the cell, particularly in service involving low current drain.

It has been proposed to fuse an enameled iron backing to the zinc plates to prevent this waste of the zinc. The simpler expedients of coating the zinc with a paint or plastic have heretofore been found to be impractical, for after a short immersion in the caustic electrolyte portions of the coating become detached.

I have discovered that the failure of such coatings is due to the fact that the amalgamated surface of the zinc does not provide a proper foundation for them. Coating materials will adhere to zinc containing no mercury. Unamalgamated zinc, however, is rarely used in present battery practice, as the advantages of the amalgamated metal are well recognized.

The present invention provides a method of treating the zinc-mercury surface to enable it to retain the coating. This method in general comprises chemical action upon the amalgamated zinc, producing a tarnished, etched, or roughened surface. Mercury appears to be substantially excluded from the treated surface and the coating adheres tenaciously to it under service conditions.

One embodiment of the invention is illus-

trated in the accompanying drawing, in which—

Fig. 1 is a vertical section through a cell having the novel protected electrodes; and

Fig. 2 is a side elevation of one of the electrodes, the coating being partly broken away.

In the drawing, reference numeral 1 denotes a perforated container for depolarizer suspended by rod 2 from the jar cover 3 and immersed in caustic electrolyte 4. Zinc plates 5 are secured in spaced relation to the container in any suitable manner, as by being threaded upon a bolt 6 which passes through the container 1. The zinc plates are treated on the sides remote from the copper oxid electrode to produce a surface 7 adapted to retain a coating 8 applied to it.

I have obtained excellent results by treating the zinc surface first with nitric acid, then with a solution of an alkaline sulfid. It is probable that the desirable character of the treated surface is due to the formation of mercury sulfids. Similar results may be secured by using other reagents. For example, a solution of an alkali metal bichromate, strongly acidified with nitric acid, is suitable. Best results are obtained when the compound formed on the zinc surface is insoluble in the caustic alkali electrolyte. When this is the case no harm will result from access of the electrolyte through any perforations or pores which may be present in the material applied to the zinc. The treated surface of the zinc should not be exposed to any considerable extent, however, as the insoluble coating is not impervious and objectionable local action would be set up.

The treating reagents may be applied to the zinc in any suitable way, as by brushing, spraying, or the like.

The coating may advantageously be pitch of high melting point, rubber cement, or equivalent material. The essential characteristics of the coating are substantial insolubility in caustic alkali and adhesion to the zinc even at the relatively high temperatures which may be reached on dissolving solid caustic in water to form the electrolyte. Low porosity is desirable. Any material having these properties will in general serve as the coating.

As compared with the coated electrodes of the prior art, those prepared by the method described herein are very efficient and inexpensive. Cells including them have 5 excellent service characteristics.

The coating may be prepared by suitable electro-chemical processes. The expression "chemical treatment" and the like, as used in the appended claims, are to be construed 10 to include such processes.

I claim:—

1. An amalgamated metal electrode having a portion roughened by chemical treatment to provide a surface adapted to retain 15 a coating.
2. An amalgamated zinc electrode having a portion superficially converted into sulfid to provide a surface adapted to retain a coating.
3. An amalgamated zinc electrode having 20 a surface chemically treated to prevent substantial access of the mercury to said surface.
4. An amalgamated metal electrode having 25 a portion chemically treated to provide a roughened surface, and a coating substantially impervious to electrolyte adherent to said surface.
5. An amalgamated zinc electrode adapted

for immersion in caustic alkali electrolyte 30 and having a portion not required for electrolytic action chemically treated to provide a roughened surface, and a protective coating material characterized by adherence to said surface notwithstanding long immersion 35 in the electrolyte.

6. The invention according to claim 5, in which the coating is pitch of relatively high melting point.

7. In the manufacture of amalgamated 40 electrodes adapted to be submerged in electrolyte and having a portion not required for electrolytic action, the step of chemically treating such portion to adapt it to retain a coating.

8. The invention according to claim 7, in which a superficial layer of sulfid is formed on the said portion of the electrode.

9. In the manufacture of amalgamated 50 electrodes adapted to be submerged in electrolyte and having a portion not required for electrolytic action, the method which comprises the chemical treatment of such portion to adapt it to retain a coating, and the application of a coating thereto.

In testimony whereof, I affix my signature.

GEORGE W. HEISE.